

Patented Aug. 18, 1953

2,649,368

# UNITED STATES PATENT OFFICE

2,649,368

## INDIUM-BISMUTH-TIN ALLOY

Albert A. Smith, Jr., Metuchen, and John L. Everhart, Linden, N. J., assignors to American Smelting and Refining Company, New York, N. Y., a corporation of New Jersey

No Drawing. Application October 7, 1950,  
Serial No. 189,045

1 Claim. (Cl. 75—134)

1

This invention relates to alloys and more particularly it relates to low fusing point alloys.

It is an object of the invention to provide cadmium-free low melting point alloys.

In accordance with the invention alloys are provided comprising 31-33% Bi, 50-52% In, 16-18% Sn and have fusing points of approximately 60° C.

It will be observed from the compositions that these alloys do not contain cadmium and accordingly they are suitable for certain applications as heat transfer media particularly in such applications where cadmium would be detrimental.

What is claimed is:

Low melting point alloys composed of 31-33% Bi, 50-52% In and 16-18% Sn. 15

ALBERT A. SMITH, JR.  
JOHN L. EVERHART.

2

References Cited in the file of this patent

### UNITED STATES PATENTS

| Number      | Name       | Date          |
|-------------|------------|---------------|
| 5 2,218,513 | Pray ----- | Oct. 15, 1940 |

### OTHER REFERENCES

French, Industrial and Engineering Chemistry, vol. 27, December 1935, pages 1464 and 1465.

10 French, Metal Industry (N. Y.), vol 35, March 1937, pages 106 and 107.

Whitehead, Metal Finishing, July 1944, pages 405-407.

262. Smith, Metal Industry, October 26, 1945, page

American Society for Metals, Cleveland, Ohio, Metals Handbook, 1948 ed., pages 744 and 745.